

# United States Patent [19]

Griffin et al.

[11] 3,816,322

[45] June 11, 1974

[54] **CORROSION INHIBITOR**

[75] Inventors: **Thomas J. Griffin; Francis E. Dollarhide**, both of Tulsa, Okla.

[73] Assignee: **The Dow Chemical Company**, Midland, Mich.

[22] Filed: Oct. 2, 1972

[21] Appl. No.: 294,327

[52] U.S. Cl..... 252/147, 252/8.55 C, 252/148, 252/388, 252/392

[51] Int. Cl..... C11d 7/32

[58] Field of Search ..... 252/147, 148, 388, 392, 252/8.55 C; 134/3

[56] **References Cited**

UNITED STATES PATENTS

|           |         |                      |           |
|-----------|---------|----------------------|-----------|
| 2,567,156 | 9/1951  | Malowan .....        | 252/392 X |
| 2,708,184 | 5/1955  | Hager et al. ....    | 252/147   |
| 3,107,221 | 10/1963 | Harrison et al. .... | 252/148   |

|           |         |                       |           |
|-----------|---------|-----------------------|-----------|
| 3,161,598 | 12/1964 | Geld .....            | 252/147   |
| 3,260,673 | 7/1966  | Fisher .....          | 252/147 X |
| 3,404,094 | 10/1968 | Keeney .....          | 252/148   |
| 3,548,945 | 12/1970 | Gidley.....           | 166/307   |
| 3,658,720 | 4/1972  | McDougall et al. .... | 252/148 X |
| 3,686,129 | 8/1972  | Loucks .....          | 252/147   |

Primary Examiner—Leon D. Rosdol

Assistant Examiner—Harris A. Pitlick

Attorney, Agent, or Firm—Bruce M. Kanuch

[57]

## ABSTRACT

Iron surfaces are protected against corrosion by aqueous acidic solutions containing a polyhydric compound or derivative thereof by dispersing into the corrosive solution which will contact the metal surface an effective amount of a heterocyclic amine, an acetylenic alcohol and an ionizable iodine containing compound.

6 Claims, No Drawings

1  
CORROSION INHIBITOR

## BACKGROUND OF THE INVENTION

U.S. Pat. No. 3,107,221 teaches that a mixture of certain amines and acetylenic alcohols inhibit corrosion of metals in contact with corrosive acids such as HCl and/or HF. However, it has been found that these inhibitors are not effective to prevent corrosion of iron by corrosive acidic solutions containing a polyhydric compound or derivative thereof, e.g. glycols and glycol ethers.

This lack of protection is especially acute with iron containing alloying amounts of such metals as chromium, nickel and the like. These iron alloys are employed to manufacture flexible oil well tubing and the like.

## SUMMARY OF THE INVENTION

Iron surfaces are protected against corrosion by acidic solutions containing a polyhydric compound or derivative thereof by dispersing into the corrosive solution an effective amount of a heterocyclic amine, e.g. pyridine, quinoline, etc., an acetylenic alcohol, and iodine anions.

The teachings of U.S. Pat. No. 3,107,221 are specifically incorporated herein by reference.

## DETAILED DESCRIPTION OF THE INVENTION

An essential constituent of the corrosion inhibitor formulation of the present invention is iodine anions. The iodine anions can be provided by organic and inorganic ionizable iodine compounds such as taught in U.S. Pat. No. 2,567,156, the teachings of which are specifically incorporated herein by reference. Included by way of example are alkali and alkaline earth metal iodine compounds, e.g. potassium iodide, sodium iodide, potassium iodate, iodo-acetic acid, ammonium iodide, hydrogen iodide, copper iodide, and the like. The particular source from which the iodine anions are derived is not critical to the practice of the invention. Iodine salts of the heterocyclic amines or acetylenic alcohols can be employed as both the source of the amine or alcohol and the iodine ions. An effective amount of the iodine compound is employed to decrease the corrosion rate of the metal to an acceptable level. As little as 0.0001 per cent by weight of the acidic solution of an iodine compound can be effective. The maximum amount is dictated by economic considerations. An acetylenic alcohol having the formula



wherein each R represents hydrogen, a C<sub>1</sub> to C<sub>15</sub> alkyl alkynyl or alkyenyl radical, or a phenyl, substituted phenyl or hydroxyalkyl alkynyl or alkyenyl radical containing from 1 to 4 carbon atoms and the α R's may be joined together to form a cyclohexyl ring is employed.

Acetylenic alcohols which can be employed include mono and polyhydric compounds such as, for example, propargyl alcohol, 1,4-butyne diol, ethynylcyclohexanol, 3-methyl-1-nonyl-3-ol, 2-methyl-3-butyn-2-ol, α-ethynyl-2,4,6-trimethylbenzyl alcohol, 2-methyl-1-pentyn-3-ol, α-ethynylbenzyl alcohol and the like.

2  
The heterocyclic amine which can be employed herein includes one or more pyridine and quinoline compounds and/or derivatives thereof.

The pyridines include pyridine and alkyl, alkynyl and alkyenyl derivatives wherein the carbon constituent can be C<sub>1</sub> to C<sub>15</sub> and can be branched or straight chained. Specific pyridines which can be employed include, for example, a mixture of alkyl pyridines having an average molecular weight of about 170.

Quinolines which can be employed are those compounds which are generally isolated from suitable coal tar distillates which have an appreciable concentration of oils boiling in the range of from about 235 to about 240° C. Compounds which are isolated in this manner include quinoline, 2-methylquinoline, 4-methylquinoline, isoquinoline, 2,8-dimethylquinoline and the like. Generally, the pyridine and quinoline compounds are employed as complex mixtures containing several species of the compounds. Quaternary salts of both pyridine, quinoline and derivatives thereof can be employed. Also, mixtures of quinolines and pyridines are useful. Specific quinoline compounds which can be employed include N-benzolquinoline chloride; 1-benzoyl-2-cyano-1,2-dihydroquinoline; 2-carboxyquinoline; 2-cyanoquinoline. Also alkyl quinoline; quinoline aldehydes; hydroquinolines, e.g. 1,2-dihydroquinoline; N-methyl-2-phenyl-1,2-dihydroquinoline quinoline methiodide; 1,2,3,4-tetrahydroquinoline; 6-nitrosotetrahydroquinoline; cis and trans decahydroquinoline; hydroxyquinolines such as 2 and 4-hydroxyquinolines; 3-carboxy-4-hydroxyquinoline; 7-iodo-8-hydroxyquinoline-5-sulfonic acid; 5-chloro-7-iodo-8-hydroxyquinoline; the copper salt of 8-hydroxyquinoline; haloquinolines such as 2 and 4 chloroquinolines; 4,7-dichloroquinoline; ethyl-4-hydroxy-7-chloro-3-quinoline carboxylate; 3-bromoquinoline; aminoquinolines such as 3-aminoquinoline; 4-aminoquinoline; 4-alkylaminoquinoline; 8-aminoquinoline; 6-methoxy-8-dialkylaminoalkylaminoquinoline; aldehydes; ketones and acids of quinoline such as 2 and 4 quinoline carboxaldehydes; quinaldaldehyde; 2-quinoline carboxylic acid; benzoquinolines such as benzo[f] quinoline; biquinoline; isoquinoline and the like.

In carrying out the present invention the constituents of the corrosion inhibitor are mixed with an aqueous solution of a mineral acid or with water which is thereafter mixed with the mineral acid. The inhibited acid solution may then be employed in oil well acidizing or industrial acid cleaning methods. The amine and acetylenic alcohol are employed in a volume ratio of about 9 to 1 to 1 to 9 amine to alcohol and employed in a total amount of from about 0.05 to about 1 per cent by volume of the acidic solution to be inhibited.

In a preferred manner of carrying out the present invention a heterocyclic amine, an iodine compound and an acetylenic alcohol are mixed together, in the range of ratios hereinbefore described, as an aqueous or hydrocarbon mixture, preferably with a surface active agent. The resulting mixture is agitated to assure complete distribution of the additives in the aqueous phase. Thereafter this mixture is mixed with an acidic solution to obtain an inhibited acid suitable for use in oil well acidizing or industrial acid cleaning methods.

Various types of surface-active agents have been found to be effective and useful in assuring the complete dispersion of the active ingredients throughout

the composition and a better contact of the inhibitor with the metallic surface. In general, any surface-active agent that is stable in aqueous acid may be used. Thus, for example, one may employ from 0.05 to 2 per cent by volume of an ionic or nonionic surface-active dispersing agent, such as an oxyethylated alkylphenol, ammonium alkylbenzene-parasulfonate, dioctyl sodium sulfosuccinate, or trimethylstearylammmonium chloride.

Various acidic solutions containing, in addition, a polyhydric compound have been found to be effectively inhibited against metal corrosion by the employment of the compositions of the present invention. Thus, mineral acids such as sulfuric, phosphoric, acetic and hydrochloric acids and the like may be effectively inhibited by employing the principles of the present invention.

Polyhydric compounds are employed in acidic solutions for various purposes. For example, in U.S. Pat. No. 3,548,945 glycol ethers are employed in conjunction with aqueous acid solutions to acidize siliceous formations. The teachings of the patent are specifically incorporated herein by reference. It is these types of aqueous acidic solutions which were found to be corrosive even in the presence of amine-acetylenic alcohol inhibitors which are taught in U.S. Pat. No. 3,107,221. The present invention overcomes this problem through the discovery that the effectiveness of these inhibitors is substantially increased by including in addition an iodine ion. Thus, acidic aqueous solutions containing polyhydric compounds such as glycols, e.g. polyglycols, ethylene glycol, glycol ethers or glycol esters, such as taught in U.S. Pat. No. 3,548,945, at col. 2, line 62 through col. 3, line 2, can be inhibited by practicing the principles of the present invention.

The inhibitors of the present invention are unique in that they are operable when employed at both low temperatures and at temperatures as high as about 275° F.

were placed in a four ounce, wide mouth bottle. An inhibitor to be tested was then mixed with the acid. After weighing the metal coupon it was placed in the acid solution. The test solution was then heated and the test coupons kept in contact with the acid solution for about 4 hours at a temperature of 250° C and 1000 psi or 120° C for 16 hours at vapor pressure. The metal coupon was removed from the acid solution at the end of the test period, cleaned, dried and reweighed. The corrosion rate was then calculated and set forth as the loss of metal in lbs/sq. ft. The various inhibitor solutions tested are set forth in the following Table I. The corrosion test data are set forth in Table II. The acid medium consisted of a mixture of 90 parts by volume of a 15 per cent by weight HCl solution and 10 parts by volume of ethylene glycol monobutyl ether.

TABLE I  
Inhibitor Formulations

| 20 | Inhibitor Code | Composition Per Cent by Weight                                                                                      |
|----|----------------|---------------------------------------------------------------------------------------------------------------------|
|    | A.             | propargyl alcohol 6.6<br>isopropyl alcohol 7.2<br>hydrocarbon solvent 56.0<br>alkylphenol ethylene oxide adduct 7.3 |
| 25 |                | alkylpyridine chlorides 12.6<br>alkylquinolinium chloride 10.3                                                      |
|    | B.             | Same as A. except alkylpyridine chloride and alkylquinolinium chloride obtained from different commercial source.   |
| 30 | C.             | kerosene 56.0<br>surfactant 7.5<br>isopropyl alcohol 7.0<br>dodecyl amine 29.5                                      |
|    | D.             | kerosene 56.0<br>surfactant 7.5<br>isopropyl alcohol 7.0<br>alkylpyridine 16.3<br>alkylquinoline 13.2               |
| 35 | E.             | kerosene 56.0<br>surfactant 7.5<br>isopropyl alcohol 7.0<br>dodecyl amine 23.0<br>propargyl alcohol 6.5             |
|    | F.             | kerosene 56.0<br>surfactant 7.5<br>isopropyl alcohol 7.0<br>propargyl alcohol 29.5                                  |

TABLE II

| Test No.  | Inhibitor | Concentration percent by wt. of acid solution | Salt and concentration                                                            | Temp °C | Corrosion rate lbs/sq. ft., iron sample 1 | 2      |
|-----------|-----------|-----------------------------------------------|-----------------------------------------------------------------------------------|---------|-------------------------------------------|--------|
| 1..... A  |           | 1.5                                           | KI (one lb. per 1 gal. of inhibitor).....                                         | 250     | 0.038                                     | 0.019  |
| 2..... B  |           | 0.1                                           | KI (one lb. per 1000 gal. of acid sol.).....                                      | 120     | 0.0074                                    | 0.0054 |
| 3..... C  |           | 0.1                                           | KI (one lb. per 1000 gal. of acid sol.).....                                      | 120     | 0.024                                     | 0.030  |
| 4..... D  |           | 0.1                                           | KI (one lb. per 1000 gal. of acid sol.).....                                      | 120     | 0.016                                     | 0.014  |
| 5..... E  |           | 0.1                                           | KI (one lb. per 1000 gal. of acid sol.).....                                      | 120     | 0.013                                     | 0.013  |
| 6..... E  |           | 1.5                                           | KI (15 lbs. per 1000 gals. acid).....                                             | 250     | 0.45                                      | 0.57   |
| 7..... F  |           | 0.1                                           | KI (one lb. per one gal. of acid).....                                            | 120     | 0.018                                     | 0.011  |
| 8..... A  |           | 1.5                                           | None.....                                                                         | 250     | 0.17                                      | 0.035  |
| 9..... A  |           | 1                                             | Na <sub>2</sub> PO <sub>4</sub> (50 lb. per 1000 gal. of acid).....               | 250     | 0.33                                      | .....  |
| 10..... A |           | 1                                             | Na <sub>3</sub> B <sub>4</sub> O <sub>7</sub> (25 lb. per 1000 gal. of acid)..... | 250     | 0.30                                      | .....  |

### EXAMPLE

Metal coupons composed primarily of iron with varying amounts of the other elements such as carbon, silicon, manganese, molybdenum, chromium, nickel, phosphorous, sulfur and zirconium were used to determine the corrosion rate of various inhibited and uninhibited HCl solutions. The following procedure was employed to determine the corrosion rate of an acidic solution. First, 100 milliliters of a test acid solution

60 An acceptable corrosion standard set for the iron sample No. 1 is less than 0.05 lb/sq. ft. at a temperature of 250° C; .02 lb/sq. ft. at a temperature of about 200° C and 0.01 lb/sq. ft. at a temperature of about 120° C. For iron sample No. 2 the acceptable corrosion rate is established to be about one half of that for sample No. 1.

What is claimed is:

1. An acidic solution inhibited to corrosion of metal which consists essentially of:

- a an acid selected from the group consisting of HCl, sulfuric, phosphoric, acetic, hydrofluoric, formic, propionic and mixtures thereof,
- b an acetylenic alcohol,
- c a heterocyclic amine,
- d an ionizable iodine compound, and
- e a water soluble polyhydric organic compound, said amine and alcohol making up from about 0.05 to about 1 per cent by weight of the composition, and further wherein said amine and said alcohol being present in said composition in a volume ratio of amine to alcohol ranging from about 9 to 1 to about 1 to 9, said ionizable iodine compound being present in an amount of at least about 0.0001 per cent of said composition, further wherein said polyhydric compound is a glycol, or a glycol ether present in an amount ranging from about 2 to about 25 per cent by volume of said acid, said acetylenic alcohol has the formula



wherein each R represents hydrogen, a C<sub>1</sub> to C<sub>15</sub> alkyl, alkynyl or alkyenyl group, a phenyl or substituted phenyl group, or a hydroxyl C<sub>1</sub> to C<sub>4</sub> alkyl, alkynyl or alkyenyl group wherein the  $\alpha$  R's may be joined together to form a cyclohexyl group, and the heterocyclic amine is pyridine or its alkyl, alkenyl or alkynyl derivatives wherein the carbon constituent can be C<sub>1</sub> to C<sub>15</sub> or a--. quinoline compound.

- 2. The composition of claim 1 wherein said ionizable

iodine compound is an alkali or alkaline earth metal iodine containing compound.

- 3. The composition of claim 1 wherein said polyhydric compound is a glycol ether.

- 5. 4. The composition of claim 1 wherein said polyhydric compound is a glycol.

5. The composition of claim 1 wherein the heterocyclic amine is selected from the group consisting of pyridine, alkyl, alkynyl or alkyenyl pyridines wherein the carbon constituent contains C<sub>1</sub> to C<sub>15</sub> or quinoline; 2-methyl quinoline; 4-methyl quinoline; isoquinoline; 2,8-dimethyl quinoline; N-benzol quinoline chloride; 1-benzoyl-2-cyano-1,2-dihydro quinoline; 2-carboxy quinoline; 2-cyano quinoline; 1,2-dihydro quinoline; N-methyl-2-phenyl-1,2-dihydro quinoline; quinoline methiodide; 1,2,3,4-tetra-hydro quinoline; 6-nitrosotetrahydro quinoline; cis and trans decahydro quinoline; 2 and 4-hydroxy quinoline; 3-carboxy-4-hydroxy quinoline; 7-iodo-8-hydroxy quinoline-5-sulfonic acid; 5-chloro-7-iodo-8-hydroxy quinoline; the copper salt of 8-hydroxy quinoline; 2 and 4 chloro quinolines; 4,7-dichloro quinoline; ethyl-4-hydroxy-7-chloro-3-quinoline carboxylate; 3-bromoquinoline; 3-aminoquinoline; 4-aminoquinoline; 4-alkylaminoquinoline; 8-aminoquinoline; 6-methoxy-8-dialkylaminoalkylaminoquinoline; 2 and 4 quinoline carboxyaldehyde; quinaldehyde; 2-quinoline carboxylic acid; benzo quinoline; biquinoline; and mixtures of such heterocyclic amines.

- 6. A method of cleaning iron surfaces which comprises contacting said surface with an acidic solution as defined in claim 1.

\* \* \* \* \*